

July 1, 1947.

G. W. RIGBY

2,423,344

PROCESS FOR STABILIZING DITHIOLYCAROLS

Filed Aug. 16, 1943



*George Wayne Rigby* INVENTOR.

BY  
*Paul J. Cullane*  
ATTORNEY

## UNITED STATES PATENT OFFICE

2,423,344

PROCESS FOR STABILIZING  
DITHIOLYCGEROLSGeorge Wayne Rigby, Wilmington, Del., assignor  
to E. I. du Pont de Nemours & Company, Wil-  
mington, Del., a corporation of Delaware

Application August 16, 1943, Serial No. 498,846

17 Claims. (Cl. 260—609)

1

This invention relates to thioglycerols, in particular to 1,2-dithioglycerol. More specifically, it relates to a process for improving the stability of thioglycerols against thermal decomposition.

2,3-dimercaptopropanol-1, hereinafter called 1,2-dithioglycerol, is a recently synthesized compound of considerable interest and usefulness, either per se, e. g., as softening agent, plasticizer, etc., or as an intermediate in chemical syntheses because of the presence, in the same molecule, of an hydroxyl group and two vicinal mercapto groups. There is, however, one property of the thioglycerols which has militated against their extensive use. This is their heat instability. This thermal instability, which was observed by the first investigator in the field [Carious, Ann. 124, 257 (1861)] is particularly noticeable with 1,2-dithioglycerol. The problem it presents is two-fold. First, distillation of crude 1,2-dithioglycerol on anything approaching a commercial scale presents extreme difficulties. Even using very small batches, very low pressure, and inert atmospheres, distillation of 1,2-dithioglycerol entails considerable losses in the form of undistillable residue. Large quantities cannot be distilled in a single operation, since, after a small amount of distillate has been collected, the residue resimifies and the bulk of the material is lost. Second, the distilled 1,2-dithioglycerol is itself also heat-unstable and, in reactions or uses involving a high temperature, decomposes to a large extent with formation of undesirable by-products and the attendant disadvantages of low yields, difficult reaction control and wasted material.

The heat decomposition of the thioglycerols is particularly severe when they are prepared by reacting the corresponding glycerol halohydrins with alkali hydrosulfides. The usefulness of this preparative method, which is intrinsically the most convenient and preferred one, is thus largely negated by the fact that the reaction product can be isolated only with great difficulty and, when isolated, is still thermally unstable.

This invention has an object the provision of a process for stabilizing thioglycerols, in particular 1,2-dithioglycerol, against thermal decomposition. Another object is to provide a process whereby 1,2-dithioglycerol can be distilled in high yields and with a minimum of side reactions from crude reaction mixtures containing it. A further object is to stabilize distilled 1,2-dithioglycerol against further heat decomposition. Other objects will appear hereinafter.

These objects are accomplished by the follow-

2

ing invention which comprises incorporating with the thioglycerol, and particularly 1,2-dithioglycerol, as a stabilizer against thermal decomposition, a member of the class consisting of ammonia, ammonium salts and amides. The invention also comprises thioglycerol compositions and particularly 1,2-dithioglycerol compositions, having a thermal decomposition factor, K (as defined hereinbelow), of not more than  $5 \times 10^{-4}$ .

According to the preferred mode of practicing the invention, there is added to the 1,2-dithioglycerol, prior to the heat treatment (e. g., distillation, high temperature reaction, etc.) about 1% by weight of aqueous ammonia, ammonium acetate or ammonium phosphate. This simple treatment is sufficient to decrease considerably the tendency of 1,2-dithioglycerol to decompose, resimify or dehydrate when heated. When the treatment is applied to the crude product obtained by reacting glycerol-1,2-dibromohydrin with sodium hydrosulfide, it greatly facilitates the isolation of the pure product since the crude 1,2-dithioglycerol so obtained cannot be distilled (except on an impractically small scale) without the use of one of the stabilizers of this invention. The mode of operation of the stabilizers proposed herein has not been satisfactorily explained. Their beneficial action is apparently not a result of the neutralization of the acidic components which may be present in crude 1,2-dithioglycerol, since bases such as piperidine or sodium bicarbonate are not only ineffective, but definitely harmful in that they actually increase the rate of thermal decomposition. Conversely, amides as a class, although not particularly basic, are excellent stabilizers.

The thioglycerols may be made by methods published in the literature. For example, the preparation of 1,2-dithioglycerol is described in Ber. 75, 13 (1942). As mentioned before, one of the most economical processes, which is also the process in which the heat decomposition is the most serious problem, is that in which a glycerol dihalohydrin is reacted with sodium hydrosulfide.

The 1,2-dithioglycerol used in the following example and tests was prepared as follows: Five hundred and sixty parts of a 15.6% methanol solution of sodium hydroxide are saturated with hydrogen sulfide at 0° C. and charged into a cooled steel autoclave together with 145 parts of glycerol-1,2-dibromohydrin. The reaction mixture is then saturated promptly with hydrogen sulfide at 100 lbs./sq. in. pressure and the mixture is heated at 65° C. for 5 hours. The contents of the autoclave

are cooled and acidified with 8% hydrochloric acid and the methanol is then removed by distillation at reduced pressure. The residue of oil and salt is taken up in water and chloroform, the layers are separated and the aqueous solution is extracted three times with additional chloroform. The combined extracts are dried over sodium sulfate and the chloroform is removed at reduced pressure, leaving an oily residue of crude 1,2-dithioglycerol.

The more detailed practice of the invention is illustrated by the following example, wherein parts given are by weight. There are, of course, many forms of the invention other than these specific embodiments.

#### EXAMPLE

To 600 parts of topped dithioglycerol, i. e., the crude reaction product left after removal of the inorganic salts and the volatile constituents as described above, are added 6 parts of ammonium acetate. The mixture is then charged into a still pot which is heated in an oil bath at a temperature of 150°-170° C. and the 1,2-dithioglycerol is distilled at a pressure of 15 mm. After a small foreshot amounting to about three parts the major part of the product distills at a temperature of 110-120° C. The distilled dithioglycerol is of high purity as shown by its physical constants:

|                    |                                                                                                            |
|--------------------|------------------------------------------------------------------------------------------------------------|
| $N_D^{25}$         | 1.5790                                                                                                     |
| $D_4^{25}$         | 1.2404                                                                                                     |
| Viscosity          | 13.5 centipoises at 25° C.                                                                                 |
| $H_2O$ solubility  | 7.8% at 25° C.                                                                                             |
| Surface tension    | 46.9 dynes/cm. at 25° C.                                                                                   |
| U. V. transmission | 86% through a 1 cm. layer at wave-length 3341, with the instrument set so that 1 cm. water transmits 100%. |

The yield amounts to 392 parts or 65% of the material charged. A viscous, non-volatile residue remains in the still pot, amounting to 186 parts or 31% of the material charged.

In contrast to these results, a sample of topped crude 1,2-dithioglycerol is distilled as described above but without the ammonia acetate. From a charge of 600 parts there is obtained 35 parts of low-boiling foreshots, 318 parts of dithioglycerol which is yellow in color and has the following physical constants:

|                    |                                                                                                              |
|--------------------|--------------------------------------------------------------------------------------------------------------|
| $N_D^{25}$         | 1.5730                                                                                                       |
| $D_4^{25}$         | 1.2352                                                                                                       |
| $H_2O$ solubility  | 6.00% at 25° C.                                                                                              |
| Surface tension    | 40.5 dynes/cm. at 25° C.                                                                                     |
| U. V. transmission | 0% through a 1 cm. layer at wave-length 3341, with the instrument set so that 1 cm. of water transmits 100%. |

and 202 parts of very viscous, non-volatile residue. The distilled dithioglycerol amounts to 53% of the material charged and the residue comprises 34% of the material charged. This shows that, in the absence of the added ammonium acetate stabilizer, the distilled product is of poor quality and is obtained in lower yield than in the presence of the stabilizer.

The remarkable increase in the heat stability of 1,2-dithioglycerol treated according to the method of this invention can readily be shown by a simple viscosity test as follows: On heating, 1,2-dithioglycerol undergoes decomposition and progressive polymerization which manifest themselves by an increase in the viscosity of the liquid.

If a sample of 1,2-dithioglycerol is heated under an inert (e. g., nitrogen) atmosphere in a glass tube at constant temperature, the relatively viscosity of the material can be determined at intervals by means of a simple viscometer, for example, a glass pipette. This viscometer is kept immersed in the liquid until a test is made. To make a measurement, the viscometer is filled with the liquid, and raised above the surface. The time

required for the liquid in the viscometer to flow, under the influence of gravity, between two graduations on the viscometer, is noted. A constant temperature for the heating and the viscosity measurement is conveniently obtained by placing the tube containing the 1,2-dithioglycerol and the viscometer in a glass jacket where it is surrounded by the vapors of a constant boiling, stable liquid maintained at its boiling point. Such a liquid may be, for example, bromobenzene, which boils at 156° C. The relative flow times, i. e., the ratios between the flow times at various time intervals and the initial flow time (all being determined at the same temperature) are independent of the viscometer used and give an accurate picture of the increase in viscosity, which in turn is an index of the progressive decomposition of the sample. For example, a sample of distilled 1,2-dithioglycerol had an initial flow time, in the viscometer employed, of 109 seconds at 156° C. After two hours at that temperature, the flow time was 157 seconds; after four hours, it was 301 seconds and, after five hours, 404 seconds. In contrast to this, distilled 1,2-dithioglycerol containing 1.25% by volume of commercial ammonium hydroxide (ammonia) and which showed an initial flow time at 156° C. of 105 seconds, had after seven hours' heating at that temperature a flow time of only 108 seconds. This shows the remarkable increase in stability resulting from the addition of a small amount of aqueous ammonia.

The influence on the heat stability of 1,2-dithioglycerol of small amounts of the stabilizers proposed herein can be shown graphically by plotting on semi logarithmic paper the heating times in minutes as abscissae and the flow times in seconds as ordinates. It is found that, after an induction period, the curve correlating heating times and flow times for each sample is essentially a straight line.

The drawing shows a set of five such curves. The middle one is that of distilled 1,2-dithioglycerol alone, i. e., the control. The considerable heat stabilizing effect of urea and ammonium chloride (1% by weight of the dithioglycerol) is shown by the two lower curves. For comparison, the two upper curves show the harmful effect caused by the use of 1% by weight of two organic bases, n-octylamine and piperidine. All measurements were made at 156° C.

Since the viscosity curve for any given sample of 1,2-dithioglycerol is a straight line (neglecting the induction period), its slope is a constant which expresses the heat stability of the sample. This constant, K, which may be called the thermal decomposition factor, is obtained by dividing the difference between the logarithms of the flow times (in seconds) at two different times  $T_2$  and  $T_1$ , by the difference (in minutes) between the same two times:

$$K = \frac{\log \text{flow time at time } T_2 - \log \text{flow time at time } T_1}{T_2 - T_1}$$

The value of the thermal decomposition factor, K, measured at 156° C. for a typical sample of distilled 1,2-dithioglycerol is  $22.8 \times 10^{-4}$ . Sam-

ples of greater stability have a smaller factor, while less stable samples have a higher factor. The following tables show the increase in heat stability resulting from the addition of 1% by weight of ammonia, various ammonium salts and various amides to distilled 1,2-dithioglycerol:

Table I

| Stabilizer (1% by weight)   | K at 156° C. $\times 10^{-4}$ |
|-----------------------------|-------------------------------|
| None                        | 22.8                          |
| Ammonium chloride           | 3.02                          |
| Urea                        | 1.43                          |
| Ammonium sulfate            | 1.30                          |
| Semi-carbazide              | 1.21                          |
| Disodium ammonium phosphate | 1.13                          |
| Benzamide                   | 1.09                          |
| Epsilon-caprolactam         | 1.03                          |
| Ammonium acetate            | 0.80                          |
| Glycine                     | 0.69                          |
| Ammonium hydroxide          | 0.56                          |
| Acetamide                   | 0.24                          |

For comparison, it is interesting to note that a number of acid-accepting agents not belonging to the class of ammonia, ammonium salts and amides have a definitely harmful effect on the heat stability of 1,2-dithioglycerol, as shown by the following table. In all cases there was added 1% by weight of acid-accepting agent.

Table II

| Acid-Accepting Agent (1% by weight) | K at 156° C. $\times 10^{-4}$ |
|-------------------------------------|-------------------------------|
| None                                | 22.8                          |
| Piperidine                          | 62.1                          |
| Sodium bicarbonate                  | 47.4                          |
| Triethanolamine                     | 44.4                          |
| Sodium methylate                    | 43.0                          |
| Ethanolamine                        | 29.0                          |
| n-Octylamine                        | 25.6                          |

The above tables refer to 1,2-dithioglycerol which has been previously distilled. The following table shows the data from viscosity measurements on a sample of stripped crude 1,2-dithioglycerol, i. e., the crude reaction product from which the inorganic salts and volatile material have been removed.

Table III

| Stabilizer (1% by weight)     | K at 156° C. $\times 10^{-4}$ |
|-------------------------------|-------------------------------|
| None                          | 160.00                        |
| Ammonia                       | 4.19                          |
| Glycine plus ammonia          | 3.14                          |
| Urea                          | 3.27                          |
| Ammonium acetate              | 3.14                          |
| Hydrogen diammonium phosphate | 2.65                          |
| Triammonium phosphate         | 2.03                          |
| Disodium ammonium phosphate   | 1.83                          |

As indicated before, the unstabilized crude reaction product cannot be distilled except in very small batches and under very low pressure. Table III shows the remarkable improvement in the heat stability of crude 1,2-dithioglycerol, as expressed by the values of K, brought about by various stabilizers.

Any organic or inorganic ammonium salt, or any carbonamide, is operable in the process of this invention. In addition to the stabilizers already disclosed, there may be mentioned ammonium fluoride, ammonium bromide, ammonium iodide, ammonium carbonate, ammonium sulfamate; the ammonium salts and amides of the aliphatic acids such as propionic, lactic, butyric, valeric, lauric, palmitic, stearic, undecylenic, oleic, and sorbic acids; of the mixed fatty acids occurring naturally in oils such as fish oil or linseed oil; of cycloaliphatic acids such as cyclo-

hexanemonocarboxylic and cyclohexanedicarboxylic acids; of aromatic acids such as benzoic, toluic, and naphthoic acids; of araliphatic acids such as phenylacetic, phenylpropionic and cinnamic acids; of polybasic acids such as oxalic, adipic, sebacic, and tartaric acids; of heterocyclic acids such as furoic and nicotinic acids; the N-mono- and disubstituted amides such as N-methylacetamide, N-ethylpalmitamide, N,N-dimethylformamide, N,N-diethylacetamide, ethyleneurea, N,N'-dimethylurea; cyclic amides such as epsilon-caprolactam; inner ammonium salts such as glycine; semi-carbazide, either as such or as the hydrochloride; biuret, etc. Mixtures of two or more stabilizers, such as ammonium hydroxide and ammonium phosphate, can be used, if desired. It is unnecessary that the stabilizer be soluble in the 1,2-dithioglycerol to any substantial extent.

Of the broad class of stabilizer disclosed, the preferred ones are those which bring the thermal decomposition factor of 1,2-dithioglycerol down to a value of  $5 \times 10^{-4}$  or less. Dithioglycerol having a thermal decomposition factor of less than  $5 \times 10^{-4}$  is particularly useful since it is quite satisfactory for use in reactions involving high temperatures. Because of their cheapness and effectiveness, ammonia and ammonium phosphate are two of the preferred stabilizers.

The stabilizers can be used in any desired amount, but it is obviously uneconomical to use more than is required for adequate stabilization. In general, it is quite unnecessary to use more than 5% by weight, and 1% has been found sufficient in the large majority of cases. Preferably, there should be used at least 0.1% of stabilizer by weight of 1,2-dithioglycerol, though quantities as small as 0.01% have a beneficial effect.

In addition to ammonia, ammonium salts and amides, a few other compounds have been found to influence favorably the heat stability of 1,2-dithioglycerol. Some of these compounds are methylamine, hexamethylenetetramine, hydroxylamine, tributylamine and a mixture of disodium hydrogen phosphate and potassium dihydrogen phosphate. However, the effect of these materials is usually not as marked as that of the ammonium salts and amides, and furthermore, such effect as they show is not general for the chemical classes to which these agents belong.

This invention has been illustrated with particular reference to 1,2-dithioglycerol. However, it is of value also with the other thioglycerols, i. e., monothioglycerol, 1,3-dithioglycerol and tri-thioglycerol.

The above description and examples are intended to be illustrative only. Any modification of or variation therefrom which conforms to the spirit of the invention is intended to be included within the scope of the claims.

What is claimed is:

1. A dithioglycerol composition containing as a thermal stabilizer therefor a member of the class consisting of ammonia, ammonium salts, and carbonamides, said composition having a thermal decomposition factor of not more than  $5 \times 10^{-4}$  said thermal decomposition factor being equal to

$$70 \frac{\log \text{flow time at time } T_2 - \log \text{flow time at time } T_1}{T_2 - T_1}$$

2. A 1,2-dithioglycerol composition containing as a thermal stabilizer therefor a member of the class consisting of ammonia, ammonium salts,

and carbonamides, said composition having a thermal decomposition factor of not more than  $5 \times 10^{-4}$  said thermal decomposition factor being equal to

$$\frac{\log \text{flow time at time } T_2 - \log \text{flow time at time } T_1}{T_2 - T_1}$$

3. A 1,2-dithioglycerol composition containing ammonia, said composition having a thermal decomposition factor of not more than  $5 \times 10^{-4}$  said thermal decomposition factor being equal to

$$\frac{\log \text{flow time at time } T_2 - \log \text{flow time at time } T_1}{T_2 - T_1}$$

4. Process of stabilizing a dithioglycerol which comprises incorporating therewith a member of the class consisting of ammonia, ammonium salts and carbonamides.

5. Process of stabilizing 1,2-dithioglycerol which comprises incorporating therewith a member of the class consisting of ammonia, ammonium salts and carbonamides.

6. Process of stabilizing 1,2-dithioglycerol which comprises incorporating ammonia therewith.

7. A dithioglycerol composition containing as a thermal stabilizer therefor a member of the class consisting of ammonia, ammonium salts, and carbonamides.

8. A 1,2-dithioglycerol composition containing as a thermal stabilizer therefor a member of the class consisting of ammonia, ammonium salts, and carbonamides.

9. A 1,2-dithioglycerol composition containing ammonia.

10. Process of stabilizing 1,2-dithioglycerol which comprises incorporating an ammonium salt therein.

11. Process of stabilizing 1,2-dithioglycerol which comprises incorporating ammonium acetate therein.

12. Process of stabilizing 1,2-dithioglycerol which comprises incorporating a carbonamide therein.

13. Process of stabilizing 1,2-dithioglycerol which comprises incorporating urea therein.

14. A 1,2-dithioglycerol composition containing, as a thermal stabilizer therefor, an ammonium salt.

15. A 1,2-dithioglycerol composition containing, as a thermal stabilizer therefor, ammonium acetate.

16. A 1,2-dithioglycerol composition containing, as a thermal stabilizer therefor, a carbonamide.

17. A 1,2-dithioglycerol composition containing, as a thermal stabilizer therefor, urea.

GEORGE WAYNE RIGBY.

REFERENCES CITED

The following references are of record in the file of this patent:

UNITED STATES PATENTS

| 30 | Number    | Name     | Date           |
|----|-----------|----------|----------------|
|    | 1,926,797 | Sutton   | Sept. 12, 1933 |
|    | 2,130,321 | Kharasch | Sept. 13, 1938 |